

1,240,549.

E. DU PONT.  
PROCESS FOR FINISHING EXPLOSIVE POWDER.  
APPLICATION FILED JULY 28, 1915.

Patented Sept. 18, 1917.



*WITNESS.*

Robt. McKittrick

INVENTOR

Ernest duPont  
BY  
Frank S. Busser  
ATTORNEY

# UNITED STATES PATENT OFFICE.

ERNEST DU PONT, OF WILMINGTON, DELAWARE, ASSIGNEE, BY DIRECT AND MESNE ASSIGNMENTS, TO BALL GRAIN EXPLOSIVES COMPANY, OF WILMINGTON, DELAWARE, A CORPORATION OF DELAWARE.

## PROCESS FOR FINISHING EXPLOSIVE POWDER.

1,240,549.

Specification of Letters Patent. Patented Sept. 18, 1917.

Application filed July 28, 1915. Serial No. 42,261.

To all whom it may concern:

Be it known that I, ERNEST DU PONT, a citizen of the United States, residing at Wilmington, county of New Castle, and State of Delaware, have invented a new and useful Improvement in Processes for Finishing Explosive Powder, of which the following is a full, clear, and exact description, reference being had to the accompanying drawings,

10 which form a part of this specification.

The object of my invention is to provide a new and improved process and apparatus whereby, in the process of glazing explosive powder, the dust that has rubbed off in the 15 smoothing operation may be removed in order that the grains may be properly polished.

A preferred construction of apparatus embodying my invention and adapted to 20 carry out my process is shown in the accompanying drawings, in which—

The two rotary tubes *a* and *b* shown in the drawings are arranged so that the outlet of one communicates with the inlet of another. Each tube may be constructed in accordance with an application filed of even date herewith by Francis I. du Pont, Serial No. 42266. Such construction is as follows: The inlet end *c* of each tube is annular, 25 enclosing an opening into which extends the discharge end of a hopper *d*. Within the tube, near its inlet end, is a section of a spiral *e*, similar to a spiral conveyer. The spiral revolves with the tube in such a direction as to convey forwardly the material delivered by the chute *d*. Even though the level of powder in the tube back of the spiral is low, the effect of the spiral is to 30 fill the tube continuously to as much higher a level as may be desired. The level to which the tube is filled is regulated by the diameter of the hole in the conical discharge end *f*.

Operating in conjunction with the tube *a* is an air-blast, *g* being a blower, *h* a chamber 45 containing a steam coil through which the air from the blower passes, and *i* a pipe extending from the chamber to the outlet end of the tube *a* and through which the hot blast passes to the interior of the tube.

50 The tube *a* is utilized for smoothing the grains of powder preparatory to polishing them. The air blast through the tube is sufficiently strong to continuously blow out the dust which has been rubbed off in the

smoothing operation. The blast of air is 55 heated in order to prevent the moisture of the air from moistening the powder and also because the polishing operation may be more successfully conducted when the powder is warm. The heated blast also is serviceable 60 in case the drying operations may have failed to thoroughly dry the powder before its introduction into the tube *a*.

The powder drops from the conical discharge end of tube *a* into the hopper at the 65 inlet end of tube *b*. Thence the powder passes into the tube *b*, in which the polishing operation is conducted. Into the hopper is also fed, preferably continuously, a polishing material such as graphite. The graphite 70 feeding device, which may be of any convenient construction, is shown as a hopper *m* having at its bottom a roller *n*, which revolves slowly and discharges the graphite, the rate of discharge being proportionate 75 to the speed of the roller. To insure the proper working of a feeder, there is provided a spider *o* which slowly revolves in the hopper and prevents the graphite from arching across.

80 From the above description it will be understood that the powder to be glazed travels continuously through the rotating tube *a*, which smooths the grains, the dust resulting from this operation being removed by 85 an air blast, and that the powder together with a polishing material, thence passes into and travels continuously through the rotating tube *b*, which is not provided with an air blast and which, by the motion of the 90 powder and polishing material one upon the other, polishes the grains.

Having now fully described my invention, what I claim and desire to protect by 95 Letters Patent is:

1. In the process of finishing explosive granular powder, causing the powder grains to have a combined longitudinal and transverse rolling movement and continuously applying and discharging powder at opposite ends of the moving stream so as to maintain substantially constant the volume of powder being treated and at the same time carry on the operation continuously.

2. In the process of finishing explosive 105 granular powder, causing the same to have a combined longitudinal and transverse rolling movement to smooth them, and at the

same time passing a current of air over the moving stream of grains in a direction opposite to their longitudinal direction of movement to remove the dust created by the 5 smoothing operation.

3. In the process of finishing explosive granular powder, causing the powder grains, together with a polishing material, to have a combined longitudinal and transverse rolling movement, whereby the powder is polished in a continuous manner. 10

4. In the process of finishing explosive granular powder, causing the same to have a combined longitudinal and transverse rolling movement to smooth them, and at the same time passing a current of air over the moving stream of grains in a direction opposite to their longitudinal direction of movement to remove the dust created by the 15 smoothing operation, and continuously supplying and discharging powder at opposite ends of the moving stream so as to maintain substantially constant the volume of powder being treated and at the same time 20 carry on the smoothing operation continuously. 25

5. In the process of finishing explosive granular powder, causing the powder grains, together with a polishing material, to have a combined longitudinal and transverse rolling movement, and continuously supply and discharge powder grains and polishing material at opposite ends so as to maintain substantially constant the volume of powder 30 being treated and at the same time carry on the polishing operation continuously. 35

6. The process of finishing explosive granular powder which consists in imparting to the same a continuous forward movement, introducing into the continuous stream of 40 moving powder a polishing material, and causing the powder, both back of and beyond the point of introduction of the polishing material to have also a transverse rolling movement, thereby, in a continuous 45 manner, first smoothing and then polishing the grains.

7. The process of finishing explosive granular powder which consists in imparting to the same a continuous forward movement, 50 introducing unto the continuous stream of moving powder a polishing material, and causing the powder, both back of and beyond the point of introduction of the polishing material to have also a transverse rolling movement, and directing a blast of artificially heated air over that part of the stream of powder back of the point of introduction of the polishing material in a direction opposite to the direction of forward travel of the powder, thereby, in a continuous 55 manner, first smoothing the grains and blowing away the dust created in the smoothing operation and then polishing the grains. 60

In testimony of which invention, I have hereunto set my hand, at Philadelphia, on this 27th day of July, 1915.

ERNEST DU PONT.

Witnesses:

M. M. HAMILTON,  
E. E. WALL.